

## UNITED STATES PATENT OFFICE

2,488,587

## PROCESS FOR TREATING ORGANIC SUBSTITUTION DERIVATIVE OF CELLULOSE TEXTILE MATERIALS

Camille Dreyfus, New York, N. Y., and George W. Seymour and George C. Ward, Cumberland, Md., assignors to Celanese Corporation of America, a corporation of Delaware

No Drawing. Application June 7, 1945,  
Serial No. 598,204

7 Claims. (Cl. 117—65)

1

This invention relates to the treatment of fabrics and relates more particularly to the treatment of fabrics made of or containing yarns having a basis of cellulose acetate or other organic derivative of cellulose whereby the heat resistance and ironing qualities of said fabrics may be improved.

An object of this invention is the provision of an improved process for the treatment of fabrics made of or containing cellulose acetate or other organic derivative of cellulose yarns whereby the safe ironing temperature thereof may be raised effectively and the hand, draping qualities and other characteristics of the fabrics may be improved.

Another object of this invention is to provide a process for raising the safe ironing temperature of fabrics made of or containing cellulose acetate or other organic derivative of cellulose yarns whereby the improvement effected is substantially permanent and resistant to the action of dry cleaning agents, and the like.

Other objects of this invention will appear from the following detailed description.

Cellulose acetate or other organic derivative of cellulose materials employed for the commercial production of filaments, yarns, threads and the like are thermoplastic. Therefore, exposure of these materials for even a relatively short time to elevated temperatures on the order of 230° C. or higher will effect a pronounced physical change therein. If exposed to temperatures above the softening point for longer periods of time, the cellulose acetate filaments will not only soften but their filamentary character will ultimately be destroyed. For example, fabrics containing cellulose acetate or other organic derivative of cellulose yarns or filaments ironed at too high a temperature become glossy and stiff due to a softening or melting of the surface filaments, and assume a wholly undesirable appearance.

We have now discovered that the ironing characteristics of textile materials made of or containing yarns of filaments having a basis of cellulose acetate or other thermoplastic organic derivative of cellulose may be greatly improved by subjecting them to treatment with an aqueous solution of boric acid and then subjecting the so treated fabric to a heat treatment. The treatment of the textile material with the boric acid solution may be effected by padding with, or dipping or rinsing in an aqueous solution, preferably containing 1 to 15% by weight of boric acid. The heat treatment to which the textile material is then subjected may involve hot calendering or mangling or decatizing. This treatment employing elevated temperatures eliminates the tendency

of a hot hand iron to stick to the fabric during an ironing operation and greatly improves the hand. The temperatures to which the treated fabric may then be safely exposed during ironing without any lustering, stiffening or the like taking place, is found to be substantially higher than in the case of untreated fabrics.

When a padding operation is used, the aqueous solution of boric acid is preferably applied to the fabric by causing the fabric to pass through the boric acid solution and then through a pair of nip rollers, the clearance between said rollers being adjusted so that the fabric retains from 75 to 125% by weight of the solution. The treated fabric is then dried in a suitable chamber through which heated air at a temperature of 85 to 100° C. is circulated.

After drying, the hand of the treated fabric is somewhat harsher than originally. This, as well as the tendency of the hand iron to stick, may be entirely eliminated by hot calendering or mangling or decatizing. When subjecting the treated fabric to mangling or hot calendering, temperatures of 110 to 150° C. and pressures of 2000 to 2500 pounds per square inch are usually employed.

The decatizing treatment employed may consist in winding the fabric onto a perforated metal drum with a heavy cotton blanket or apron so that a layer of the cotton blanket or apron alternates with each layer of the fabric. Steam at a pressure of the order of 10 pounds per square inch or more is then passed through the fabric for 3 to 5 minutes, whereby the temperature of the fabric is raised to 95 to 100° C., thereupon the steam is shut off and vacuum is applied to cool the fabric and remove any condensed water present.

The cellulose acetate or other organic derivative of cellulose fabric obtained after treatment in accordance with our novel process may then be dry-cleaned and the improved properties of the fabric are wholly retained without being in any way impaired. Inasmuch as the boric acid is water-soluble, washing will, of course, remove the latter and cause the heat-resistant properties of the fabric to revert back to substantially the original properties observed prior to treatment.

In order further to illustrate our invention but without being limited thereto, the following examples are given:

## Example I

A cellulose acetate fabric of taffeta weave is padded with a 15% aqueous solution of boric acid at 85° C., the fabric being permitted to retain

about 100% by weight of the solution. The padded fabric is then dried with air heated to 100° C. in a suitable drying chamber. The fabric obtained is entirely unaffected by ironing with a hand iron at a temperature of 220° C. but the iron exhibits a pronounced tendency to stick thereto. This may be entirely eliminated by our novel heat treatment comprising hot calendering under a pressure of 2000 to 8000 pounds per square inch at a temperature of 110 to 130° C. or decatizing with steam at a temperature of 90 to 110° C. When the heat-treated fabric is given 20 strokes with an iron heated to 280° C. no sticking is observed and no change in the physical appearance of the fabric takes place. Fabric to which no boric acid has been applied and given the 20 stroke ironing test with the iron at 220° C. undergoes a considerable degree of physical change due to a softening or melting of the cellulose acetate filaments.

*Example II*

A cellulose acetate tricot fabric is padded with a 5% aqueous solution of boric acid at 38° C., the fabric being permitted to retain about 100% by weight of the solution. The padded fabric is dried in a suitable drying chamber with air heated to 110° C. The dried fabric is decatized at 95 to 110° C. The treatment comprises winding the fabric on a perforated metal drum together with a cotton apron so that the cotton apron lies between each layer of the fabric and passing steam at 10 pounds per square inch pressure through the fabric for 5 minutes. The flow of steam is then halted and vacuum is applied to cool the fabric and remove condensed water. The treated fabric is entirely unaffected by allowing a hand iron at 250° C. to rest thereon in a stationary position for 10 seconds. Untreated fabric becomes stiffened and glazed under the 10 second stationary iron test at 250° C. With the iron at 270° C., the treated fabric becomes only slightly stiffened while untreated fabric undergoes such a degree of change during the 10 second test period as to glaze and stick to the heated surface of the iron.

Other methods of applying the boric acid solutions may be used. Thus garments made of fabrics comprising organic derivative of cellulose yarn after they are laundered either at home or in commercial laundries may be given a final rinse in the boric acid solution and then subjected to hydro-extracting or vacuum-extracting and then mangled. Thereupon, the garments may be ironed with a reasonably hot iron without danger of causing stiffening or glazing.

An important use of this invention is in connection with the treatment of fabrics made of or containing organic derivative of cellulose fibres that are used for the manufacture of men's or women's suits or coats. During the manufacture of such garments, the fabrics are subjected to many smoothing operations usually by means of Hoffmann presses or other presses wherein steam is passed through the fabric. Also after these garments are made, they are pressed by such presses both by the manufacturer and by tailors and dry-cleaners. When outer fabrics made of or containing cellulose acetate material whether in the form of continuous filaments or staple fibers and/or linings made of such cellulose acetate material are used, often glazing of the material results. However, if such fabrics or garments made of such fabric are treated in accordance with this invention, the ironing point

is raised sufficiently high to permit the safe use of such presses.

While our invention has been more particularly described in connection with the treatment of fabrics having a basis of yarns of cellulose acetate, it is to be understood that equally desirable results are obtained when treating fabrics having a basis of other organic derivatives of cellulose. Examples of other organic derivatives of cellulose are cellulose esters, such as cellulose propionate, cellulose butyrate, cellulose acetate-propionate and cellulose acetate-butyrate or cellulose ethers, such as ethyl cellulose or benzyl cellulose.

The expression "organic substitution derivative of cellulose" as employed in the claims is to be construed as including within its scope only cellulose ethers and cellulose esters of fatty acids.

It is to be understood that the foregoing detailed description is given merely by way of illustration and that many variations may be made therein without departing from the spirit of our invention.

Having described our invention what we desire to secure by Letters Patent is:

1. Process for improving the ironing properties of organic substitution derivative of cellulose textile materials and articles made therefrom, which comprises treating the same with an aqueous solution of boric acid, drying the material, and then subjecting the so treated material to a heat treatment at a temperature of at least 110° C. under a pressure of at least 2000 pounds per square inch.

2. Process for improving the ironing properties of cellulose acetate textile materials and articles made therefrom, which comprises treating the same with an aqueous solution of boric acid, drying the material, and then subjecting the so treated material to a heat treatment at a temperature of at least 110° C. under a pressure of at least 2000 pounds per square inch.

3. Process for improving the ironing properties of organic substitution derivative of cellulose textile materials and articles made therefrom, which comprises treating the same with a 1 to 15% aqueous solution of boric acid, drying the material, and then subjecting the so treated material to a heat treatment at a temperature of at least 110° C. under a pressure of at least 2000 pounds per square inch.

4. Process for improving the ironing properties of cellulose acetate textile materials and articles made therefrom, which comprises treating the same with a 1 to 15% aqueous solution of boric acid, drying the material, and then subjecting the so treated material to a heat treatment at a temperature of at least 110° C. under a pressure of at least 2000 pounds per square inch.

5. Process for improving the ironing properties of organic substitution derivative of cellulose textile materials, which comprises applying an aqueous solution of boric acid to said organic derivative of cellulose textile materials, drying the materials, and subjecting the materials to a heat treatment at a temperature of 110 to 150° C. under a pressure of at least 2000 pounds per square inch whereby the safe ironing temperature of the textile materials is substantially raised and the ironing qualities improved.

6. Process for improving the ironing properties of cellulose acetate textile materials, which comprises applying an aqueous solution of boric acid to said cellulose acetate textile materials, drying

the materials, and subjecting the materials to a heat treatment at a temperature of 110 to 150° C. under a pressure of at least 2000 pounds per square inch whereby the safe ironing temperature of the textile materials is substantially raised and the ironing qualities improved.

7. Process for improving the ironing properties of cellulose acetate textile materials, which comprises applying a 1 to 15% aqueous solution of boric acid to said cellulose acetate textile materials, drying the materials, and subjecting the materials to hot calendering at a temperature of 110 to 130° C. under a pressure of between 2000 to 8000 pounds per square inch whereby the safe ironing temperature of the textile materials is substantially raised and the ironing qualities improved.

CAMILLE DREYFUS.  
GEORGE W. SEYMOUR.  
GEORGE C. WARD.

20

## REFERENCES CITED

The following references are of record in the file of this patent:

## UNITED STATES PATENTS

| Number    | Name          | Date          |
|-----------|---------------|---------------|
| 1,959,350 | Ellis         | May 22, 1934  |
| 2,022,411 | Dreyfus       | Nov. 26, 1935 |
| 2,036,854 | Dickie et al. | Apr. 7, 1936  |
| 2,038,723 | Dreyfus       | Apr. 28, 1936 |
| 2,072,253 | Ellis et al.  | Mar. 2, 1937  |
| 2,121,005 | Bener         | June 21, 1938 |